

1

3,340,059

DIFFUSION TRANSFER PROCESS FOR  
PRODUCING SILVER-FREE AZO DYE  
IMAGES

Otto Boes, Neu-Isenburg, Germany, assignor to E. I. du Pont de Nemours and Company, Wilmington, Del., a corporation of Delaware  
No Drawing. Filed Sept. 27, 1963, Ser. No. 311,980  
Claims priority, application Germany, Feb. 27, 1963,

A 42,450

6 Claims. (Cl. 96—29)

This invention pertains to a novel process for producing silver-free images from photographic silver images by image-true contact transfer of a compound to an image acceptor film containing a reagent suitable for coupling.

An object of this invention is to provide new image-forming processes. A related object is to provide new processes for forming and transferring images. A further object is to provide such processes which are simple and dependable. Still further objects will be apparent from the following description of the invention.

According to the invention, a photographic silver image is treated with a solution of a diazonium compound in the presence of a substance having catalytic activity and the diazonium compound is transferred, true to the image, to an image acceptor film which is placed in intimate contact with the original silver image. The process of image formation takes the following course:

In treating the silver image, e.g., a developed silver image in an original photographic silver halide emulsion layer, with a diazonium compound solution, the latter, under the catalytic influence of suitable additives, is decomposed at points containing image silver, with formation of noncoupling degradation products. At points free from image silver, on the other hand, in the reverse areas or non-developed areas of the layer the diazonium compound is retained unchanged. By pressing the treated layer against the surface of an image acceptor element, e.g., paper or film, the diazonium compound can be transferred thereto. There is then formed in the image acceptor element, by coupling the diazonium compound with a re-

2

agent which is present in that film, an azo dye image with gradation opposite to that of the original, i.e., if the start is made with an ordinary photographic negative, then a positive image is obtained after the transfer, whereas when a positive is used as the original a negative image is obtained by diffusion.

Not only half-tones but also line negatives and screen images can serve as originals, and their base may consist of the usual transparent or opaque materials, i.e. film base or paper.

Chloride, thiocyanate, bromide and iodide ions have been found particularly suitable for use as additives which effect the catalytic decomposition of the diazo compound by the image silver, the catalytic activity of the specified ions being in ascending order as listed. In practice, this rising activity results in an apparent increase in speed and contrast. Thus, when iodide ions are used, the apparent speed is higher and the pictures exhibit high contrast, whereas when chloride ions are used relatively lower speed and contrast are obtained. The choice of a suitable catalyst for each case depends on the character of the original as well as on the requirements imposed on the finished picture, and can be easily decided from case to case by one skilled in the art.

Suitable compounds that will provide the ions referred to above include sodium and potassium chloride, bromide, iodide and thiocyanate which are illustrated in the examples. Mixtures of two or more of these compounds can be used. Other useful compounds are: the corresponding magnesium, calcium, strontium and barium salts and mixtures of two or more of the foregoing salts.

In addition, there is the possibility of influencing the sensitivity and gradation of the picture to a certain extent by varying the quantity of catalyst.

The catalytically active substances may be added to the diazonium solution singly or in combination. Practically all coupling reagents and diazonium salts which are capable of azo coupling are suitable for carrying out the processes, so that a very wide selection of dyes is available. Usable compounds are listed, for example, in the following tables:

TABLE I

| No.   | Coupling Reagent | Color          |
|-------|------------------|----------------|
| 1.... |                  | Yellow.        |
| 2.... |                  | Bright yellow. |
| 3.... |                  | Yellow.        |



5  
TABLE I—Continued

| No.   | Coupling Reagent | Color          |
|-------|------------------|----------------|
| 14... |                  | Purple.        |
| 15... |                  | Bluish red.    |
| 16... |                  | Purple.        |
| 17... |                  | Purple.        |
| 18... |                  | Bright yellow. |
| 19... |                  | Orange.        |
| 20... |                  | Red.           |

TABLE II

| No.  | Coupling Reagent | Color      |
|------|------------------|------------|
| 1... |                  | Pink.      |
| 2... |                  | Red-brown. |
| 3... |                  | Red.       |
| 4... |                  | Purple.    |
| 5... |                  | Orange.    |

| No. | Coupling Reagent | Color       |
|-----|------------------|-------------|
| 6   |                  | Purple.     |
| 7   |                  | Purple.     |
| 8   |                  | Pink.       |
| 9   |                  | Pink.       |
| 10  |                  | Bluish red. |
| 11  |                  | Orange.     |
| 12  |                  | Purple.     |
| 13  |                  | Pink.       |
| 14  |                  | Red.        |
| 15  |                  | Red.        |
| 16  |                  | Pink.       |
| 17  |                  | Bluish red. |
| 18  |                  | Blue.       |
| 19  |                  | Purple.     |

The gelatin content of suitable acceptor layers can vary from 25 to 50 g. gelatin per liter of solution.

According to a particularly advantageous embodiment, diazosulfones are used as diazonium compounds, these being known as stable solid substances, solutions of which have relatively high stability.

The new method yields silver-free images or copies in the most varied colors, the tint depending solely on the choice of diazonium compound and of the reagent or dye coupling agent present in the acceptor film. Additional broadening of the color range can be obtained by using a blend of different dye coupling agents in the acceptor film.

A gelatin film, for example, may be used as the acceptor layer, which contains a reagent capable of azo coupling and may be applied to any desired film base, e.g., paper, a cellulose ester or the like. Of course, other water-permeable colloid binding agents and film-forming materials may be used instead of gelatin as the vehicle,

such as polyvinyl alcohol, polyvinyl acetate, polyvinyl acetals, polyesters, etc. The reagents are incorporated in the film by methods known in the art, in which connection it has been found advisable to use the reagents in a diffusion-resisting form. It is desirable to coat the surface of the acceptor film containing the reagent capable of azo coupling with a thin protective layer of a water-permeable colloid, e.g., gelatin, sodium alginate, etc.

The process according to this invention is characterized by a number of advantages. Thus, it is possible to make one or more copies in a very short time from a silver-containing original without needing copy-making illumination. When making a number of copies it is well to wash the original between times, since the silver image may sometimes be attacked during prolonged action of the processing solution.

Copies may be made in ordinary daylight, so it is not necessary to provide a dark room. The requisite processing time for making a copy is relatively short, since in

ordinary cases only a single bath is necessary. In many cases washing of the copy may be omitted, so that it comes out almost dry. Gradation of images can be varied within wide limits according to requirements and depends chiefly on the kind and concentration of catalyst employed, on the coupling properties of the diazonium compound and on choice of a suitable coupling reagent. For each case the optimum values can be ascertained very quickly by a simple series of tests. The examples set forth below should serve to explain the invention in greater detail:

#### Example 1

A gelatin solution containing, per liter, 6 g. of dye coupling agent No. 4 of Table I is coated in the customary manner on a transparent film base. This material serves as the acceptor film.

A normal negative silver image is treated 30 seconds in a solution having the following composition:

|                                      |       |     |    |
|--------------------------------------|-------|-----|----|
| Water                                | liter | 1   | 20 |
| Diazonium compound No. 7 of Table II | g     | 10  |    |
| Potassium bromide                    | g     | 25  |    |
| Sodium acetate                       | g     | 25  |    |
| Glacial acetic acid                  | ml    | 2   |    |
| N-methyloleyltaurine                 | g     | 0.2 | 25 |

The clinging treatment solution is stripped from the silver image and the negative is pressed on the acceptor film with a squeegee. After 15 seconds the acceptor film is stripped away from the silver image. It contains a yellow positive transparency of the black-and-white negative. The negative is washed with water and dried. It is practically unchanged. If the dye coupling agent in the acceptor film is replaced by one of the coupling agents listed in Table I, then, by otherwise identical processing, positive images are obtained in the colors stated in the table. When coupling agents 18-20 are used, then the acceptor film, after stripping from the silver image, is given an additional treatment of 1 minute in 1% sodium carbonate solution to force formation of the dye.

#### Example 2

A half-tone negative on ordinary lithographic film serves as the original. A gelatin film on a transparent base is used as the acceptor film. It contains coupling agent No. 14 of Table I. Processing remains the same as in Example 1. The treatment solution has the following composition:

|                      |       |     |    |
|----------------------|-------|-----|----|
| Water                | liter | 1   | 50 |
| Diazonium compound   | g     | 10  |    |
| Potassium bromide    | g     | 25  |    |
| Sodium acetate       | g     | 25  |    |
| Glacial acetic acid  | ml    | 2   |    |
| N-methyloleyltaurine | g     | 0.2 | 55 |

If the diazonium compounds specified in Table II under Nos. 1-14 are introduced, positive transparencies are obtained in the colors there cited.

#### Example 3

The same original is employed as in Example 2. The acceptor film is prepared as follows: A gelatin solution is coated on an ordinary paper base; each liter of solution containing 6 g. of dye coupling agent No. 16 of Table I. A top-coat is coated on this gelatin film from a solution of the following composition:

|                            |       |   |    |
|----------------------------|-------|---|----|
| Water                      | liter | 1 | 60 |
| Sodium alginate            | g     | 5 |    |
| Rapid wetting solution, 4% | ml    | 5 | 70 |

Processing: Bath time for the silver image, 20 seconds. Contact with the acceptor film, 15 seconds.

A stock solution, to which another catalyst is added for each image, is used as the treatment bath.

#### Stock solution:

|                                      |       |     |
|--------------------------------------|-------|-----|
| Water                                | liter | 1   |
| Diazonium compound No. 2 of Table II | g     | 10  |
| Sodium acetate                       | g     | 25  |
| Glacial acetic acid                  | ml    | 2   |
| N-methyloleyltaurine                 | g     | 0.2 |

#### Catalyst:

|                                    |       |
|------------------------------------|-------|
|                                    | Grams |
| Image 1—Sodium chloride            | 50    |
| Image 2—Potassium thiocyanate      | 25    |
| Image 3—Potassium bromide          | 25    |
| Image 4—Sodium chloride+1.25 g. KI | 4     |
| Image 5—Sodium chloride+2.5 g. KI  | 25    |
| Image 6—Sodium chloride+3.75 g. KI | 12.5  |
| Image 7—Potassium iodide (KI)      | 5     |

In all seven cases a purple positive is obtained. Sensitivity and gradation of the images increase from image 1 to 7. That is, catalytic activity rises in the sequence chloride, thiocyanate, bromide, iodide.

#### Example 4

An ordinary silver image on photographic paper is used as the original. It is treated for 20 seconds with the following solution:

|                                      |       |     |
|--------------------------------------|-------|-----|
| Water                                | liter | 1   |
| Diazonium compound No. 7 of Table II | g     | 10  |
| Potassium iodide                     | g     | 5   |
| Sodium acetate                       | g     | 25  |
| Glacial acetic acid                  | ml    | 2   |
| N-methyloleyltaurine                 | g     | 0.2 |

Processing: After stripping off the bath liquid the paper image is pressed 15 seconds against the acceptor film described in Example 1. If the potassium iodide in the treatment bath is replaced by 25 g. potassium thiocyanate, a yellow negative with substantially flatter gradation is obtained.

#### Example 5

A screen negative on ordinary lithographic film is used as the original. A gelatin film on a transparent base, the dye coupling agent being compound No. 16 of Table I, is used as acceptor film. The treatment solution has the following composition:

|                                      |       |     |
|--------------------------------------|-------|-----|
| Water                                | liter | 1   |
| Diazonium compound No. 3 of Table II | g     | 10  |
| Potassium bromide                    | g     | 25  |
| Sodium acetate                       | g     | 25  |
| Glacial acetic acid                  | ml    | 2   |
| N-methyloleyltaurine                 | g     | 0.2 |

Processing is as usual, with bath time 20 seconds and contact time 15 seconds between original and acceptor film. A red positive screen image is obtained.

#### Example 6

The same original is used as in Examples 2 and 3, with the acceptor film described in Example 5. The requisite treatment solution is prepared as follows:

Solution A: 2.9 g. of the amine corresponding to diazonium compound No. 18 of Table II is dissolved in 20 ml. of 5% hydrochloric acid and diazotized in the usual way by adding a solution of 0.7 g. sodium nitrite in 5 ml. water. The resulting diazonium salt solution is adjusted to pH 6 by adding 10% sodium hydroxide solution and is then made up to 50 ml. with water.

To prepare the completed treatment solution there is then added the following Solution B:

|                      |    |      |
|----------------------|----|------|
| Water                | ml | 50   |
| Potassium bromide    | g  | 2.5  |
| Sodium acetate       | g  | 2.5  |
| Glacial acetic acid  | ml | 0.2  |
| N-methyloleyltaurine | g  | 0.02 |

The original is treated 30 seconds with this solution and, after removing excess solution, the wet surface is brought

into contact with the acceptor film for 20 seconds. The original is stripped off and the acceptor film is immediately treated for 1 minute with 0.5% sodium carbonate solution. The acceptor film is then washed with water and dried. A blue positive image is obtained. The corresponding ready A-solutions were also obtained from the diazonium salts listed in Table II as Nos. 15-17 and 19, by diazotizing the amines. They were introduced as treatment baths after adding the same B-solutions with the same material and same processing. This gave positive images in the colors stated in Table II. After treatment of the acceptor film with sodium carbonate solution was not necessary with these diazonium salts.

An advantage of the present invention is that it provides a simple and practical process for forming azo dye images in a separate element.

Another advantage of the invention is that it is possible to prepare one or several prints from an original copy containing silver within the shortest time and without any printing exposure being necessary. A further advantage is that production of the prints may take place in normal daylight, so that a dark room is unnecessary. A still further advantage of the invention is that a single treating bath only is required, so that prints can be made in a relatively short time, usually about one minute.

I claim:

1. A process for making silver-free negative copies from photographic silver images of a photographic element, characterized in that the silver image is treated with a solution of a diazonium compound capable of coupling, said solution being free from strong acid and initially

containing at least one ion selected from the group consisting of chloride, bromide, iodide and thiocyanate ions, after which the unchanged diazonium compound occurring at points free from image silver is imparted by contact transfer to an image acceptor element containing at least one reagent capable of azo coupling whereby an azo dye image is formed.

2. A process according to claim 1, characterized in that a diazosulfone is used as the diazonium compound.

3. A process according to claim 1, characterized in that the silver image original is washed with water after the contact transfer and the contact transfer step is repeated.

4. A process according to claim 1 wherein the silver image is in a gelatin layer and the image acceptor element has an acceptor surface of gelatin, which contains the reagent capable of azo coupling.

5. A process according to claim 1 wherein the solution of the diazonium compound is slightly acidic.

6. A process according to claim 1 wherein the solution of the diazonium compound is slightly acidic and the contact transfer is effected under slightly alkaline conditions.

#### References Cited

#### UNITED STATES PATENTS

|           |         |               |       |       |
|-----------|---------|---------------|-------|-------|
| 2,271,176 | 1/1942  | Gaspar        | ----- | 96-54 |
| 2,386,167 | 10/1945 | Murray        | ----- | 96-3  |
| 2,465,760 | 3/1949  | Sprung et al. | ----- | 96-91 |
| 2,747,999 | 5/1956  | Yutzy et al.  | ----- | 96-29 |

30 J. TRAVIS BROWN, *Acting Primary Examiner.*